

3,330,769

## METAL CLEANING

Michael Golben, Maplewood, and John W. Pearson, Mendota Heights, Minn., assignors to Minnesota Mining and Manufacturing Company, St. Paul, Minn., a corporation of Delaware  
No Drawing. Filed Jan. 23, 1964, Ser. No. 339,606  
5 Claims. (Cl. 252—136)

This invention relates to the cleaning of metal parts prior to the application of an overcoating material. It particularly relates to the cleaning of metal parts prior to the application of a metal by mechanical plating.

In recent years mechanical plating has replaced electroplating in many installations, especially where manufacturers are concerned with relatively small parts. In mechanical plating the parts are first cleaned to remove metal oxide, oil, and dirt, etched, and then placed in a tumbling barrel in the presence of finely divided metal powder, a promoter chemical, and, generally, impact media. As the tumbling barrel is rotated or otherwise agitated, the metal powder is squashed against the surface of the parts, forming a continuous coat. Even though the mechanical plating process is convenient and reduces the floor space required, equipment to clean the surface before plating has still occupied a disproportionate amount of the manufacturers' facilities.

For many years prior to my invention the conventional way to clean a metal surface has been a multi-step batch operation. Parts to be cleaned were first degreased to remove oil and organic contaminants, either by exposing them to trichloroethylene vapor or by immersing them in a tank of caustic solution. The degreased parts were then removed, rinsed in a second tank, removed, subjected to a descaling, or oxide-removing, acid pickle treatment by immersing them in a third tank, removed and again rinsed, often in a fourth tank. The tanks occupy considerable floor space, thereby inherently increasing the cost of the process. This cleaning operation also requires maintaining a continual check on the strength and contamination of the treating baths, and the open tanks represent a serious danger to personnel. Further, where high-carbon steel, or inadequately degreased, parts are pickled, the inorganic pickling acids often leave a carbon smut on the metal surface, making it extremely difficult to obtain uniform coverage of an overcoating material. In addition, acid pickling tends to trap hydrogen in the metal lattice, making the metal more brittle (i.e., hydrogen embrittlement), frequently resulting in breakage of a cleaned and subsequently electroplated part.

The present invention is believed to provide for the first time a unitary "one-shot" process for cleaning metal parts to be plated, thereby effecting a great economy in both cleaning time and requisite plant space. The process is convenient, eliminating the need for the constant careful maintenance of several treating baths and the transfer of parts from one bath to another. It is simple and inexpensive, producing consistent and predictable results. In accordance with the invention, the metal parts to be cleaned are placed in a container (which may be the same barrel used in mechanical plating) and a relatively small amount of aqueous cleaning solution, and, preferably, impact media are added. The parts and solution are agitated until the parts are cleaned, after which the cleaning solution is flushed away, leaving the cleaned, degreased, descaled, desmutted, etched parts ready for plating. By discarding the used cleaning solution—which is not economically feasible in a dip cleaning method—contamination is avoided, and quality control is facilitated. For cleaning parts by this unique "one-shot" method, a new and useful metal cleaning composition has been devised, comprising a combination of ingredients

which facilitates the practice of the process. This combination quickly and simultaneously effects the diverse and heretofore separate functions of degreasing, descaling, desmutting, and etching, while essentially eliminating the problem of hydrogen embrittlement. The cleaning composition comprises a water-soluble mixture of metal oxide-removing acid, hydrogen embrittlement inhibitor, and surfactant having the combined properties of metal wetting, oxide scale and dirt detergency, and oil emulsification.

The scale-removing acid used in the cleaning solution may be either mineral or organic, the former being relatively inexpensive and the latter being both easier to control and less corrosive at room temperature. Descaling and etching 10,000 grams of typical metal parts requires enough acid to supply between 1 and 5 grams of "available" hydrogen ion. Either monobasic or polybasic acids may be employed, but for purposes of this invention a hydrogen ion is considered to be "available" if it has an dissociation constant of at least  $10^{-6}$ . In order to minimize hydrogen embrittlement, I also prefer to include a hydrogen embrittlement inhibitor. Whether or not an inhibitor works with the particular acid used can be determined empirically by known procedures, of the type described in the specific example following.

Generally speaking, the required range of properties possessed by the surfactant can best be obtained by blending surfactants which are similar in ionic nature but different in surface-active characteristics. One recognized way to classify surface active agents is to establish their hydrophilic-lipophile balance (HLB), a trial and error procedure for which has been discussed at length by William C. Griffin; see, e.g., the Journal of the Society of Cosmetic Chemists, vol. I (1949), pages 311-326 and vol. V (1954), pages 249-256. A somewhat more sophisticated technique is to establish  $\phi_1$  (the ratio of the volume of oil to volume of water at the inversion point between oil-in-water and water-in-oil emulsions) and, from known values, graphically determine the HLB; see pages 378-383 of *Interfacial Phenomena*, J. T. Davies and E. K. Rideal (1961) Academic Press, New York, London.

Surfactants are molecules having a hydrophilic portion and a hydrophobic, or lipophilic, portion, so that in another sense the HLB number is related to the ratio between hydrophilic groups and lipophilic groups in the molecule. Those surfactants in which the lipophilic groups are dominant tend to be oil-soluble and hence are extremely effective in wetting surfaces which may be contaminated with organic materials, e.g., oils; such surfactants tend to have an HLB value of 5 or less. Surfactants in which the hydrophilic and lipophilic groups are roughly balanced have an HLB value in the proximate range of 12 to 17 and tend to function as detergents if their molecular weight is relatively low and as emulsifiers if their molecular weight is relatively high. Surfactants in which the lipophilic groups are dominant have an HLB value of more than 17 and function effectively as dispersants for carbonaceous or other materials.

In the preferred practice of this invention a mixture of surfactants is employed. One surfactant—a wetting agent which loosens oil and dirt and aids the acid in uniformly contacting the metal oxide scale—has an HLB value in the range of 1 to 5. Another surfactant—a detergent which aids in suspending dirt and scale—has an HLB value in the range of 12 to 17, and a third surfactant—an emulsifier which emulsifies residual oils—has an HLB value in the range of 12 to 17. Desirably, a fourth surfactant—a dispersant which prevents particle agglomeration and redeposition and which has an HLB value greater than 17—is also present.

As indicated in the preceding paragraph, emulsifying ability is a requisite for the composition of this inven-

tion. Oftentimes parts to be cleaned are supplied in very oily condition; for example, 10,000 grams of metal articles may include 150 grams or more of oil. As a convenient way to predict the emulsifying ability of a surfactant, the  $\phi_i$ , and therefrom the HLB, is determined with an emulsifying machine substantially like that described on pages 378 et seq. of the Davies and Rideal book, previously mentioned. In this machine oil<sup>1</sup> and water are pumped through flow gauges from separate reservoirs at controlled rates and fed between two polymethyl methacrylate shearing plates. A stream of emulsion impinges on a polymethyl methacrylate window; a continuous white film appears if the oil phase is continuous, and white drops appear if the water phase is continuous. A precise way of determining the inversion point involves measuring the electrical conductivity of the emulsion, which decreases sharply as the change from water-in-oil to oil-in-water occurs, and conversely increases sharply as the change from oil-in-water to water-in-oil occurs. Flow rates are adjusted to establish the oil:water ratio,  $\phi_i$ , at phase inversion.

As a further aid to understanding the invention, a presently preferred composition and its method of preparation will now be described. All parts are by weight unless otherwise noted.

#### EXAMPLE

##### *Hydrogen embrittlement inhibitor*

To 50.2 parts of de-ionized water is added 32.0 parts of a water-soluble high molecular weight polyoxyethylene glycol. The charge is heated to 120° F. and maintained at that temperature until all the polyoxyethylene glycol has been dissolved and a uniform solution has resulted. The temperature is then lowered to 75° F., at which time the following ingredients are added: 4.8 parts of concentrated hydrochloric acid, 6.5 parts of o-toluidine, and 6.5 parts of 37% formaldehyde, and the reaction kettle sealed. When the exothermic reaction has ended, the charge is heated briefly to 120° F., cooled to 85° F. and drained from the container. This composition is hereinafter referred to as "Composition A."

##### *Preparation of metal cleaning composition*

To a stainless steel kettle is charged 84.4 parts of 70% glycolic acid, 1.8 parts of "Pluronic L-64," and 1.8 parts of "Pluronic L-101." Agitation is commenced and 1.8 parts of "Pluronic P-85" and 1.8 parts of "Pluronic P-104," both normally solid materials which have been previously heated to render them fluid, are added. Mixing is continued until the composition is uniform, at which time 4.4 parts of "Composition A" is slowly added. Mixing is continued until the solution is completely uniform. The final composition has a specific gravity of 1.23.

The "Pluronics" referred to in the preceding paragraph are heat- and acid-stable, nontoxic non-ionic surfactants made by adding propylene oxide to propylene glycol in sufficient amount to form a hydrophobic nucleus, and thereafter graft polymerizing ethylene oxide on each end of the polyoxypropylene nucleus to form two hydrophilic polyoxyethylene chains. The greater the molecular weight of the nucleus for a given polyoxyethylene:polyoxypropylene ratio, the greater the hydrophobic (or lipophilic) nature of the surfactant; conversely, the greater the length of the polyoxyethylene chains for a given polyoxyethylene:polyoxypropylene ratio, the more hydrophilic the surfactant. "Pluronic L-64" is a liquid which has a polyoxypropylene nucleus having an average molecular weight of about 1,750, polyoxyethylene making up approximately 40% of the total weight of the molecule; this surfactant has an HLB value of 15 and is useful as a carbon soil remover. "Pluronic L-101" is a liquid having a polyoxypropylene nucleus with an average molecular weight of

about 3,250, polyoxyethylene making up approximately 10% of the total weight of the molecule; this surfactant has an HLB value of about 1, is strongly lipophilic, and functions as a wetting agent and defoamer. "Pluronic P-85" is a paste having a polyoxypropylene nucleus with an average molecular weight of about 2,250, polyoxyethylene making up approximately 50% of the total weight of the molecule; this surfactant has an HLB value of approximately 16 and functions primarily as a detergent. "Pluronic P-104" is a paste having a polyoxypropylene nucleus with an average molecular weight of approximately 3,250, polyoxyethylene making up approximately 40% of the total weight of the molecule; this surfactant has an HLB value of approximately 13 and is particularly useful as an emulsifying agent.

The cleaning composition just described is extremely useful for a wide range of metal cleaning operations. Thus, although metal parts vary in surface area and amount of scale, and although such parts are often not completely drenched with oil, this composition is suitable for cleaning operations in which the worst reasonably anticipated conditions might be encountered.

The novel one-shot method taught herein provides simultaneous mechanical and chemical cleaning of metal parts which are to be subsequently overcoated. The parts are placed in an aqueous descaling and degreasing composition, which is then vigorously agitated while the parts are being mechanically cleaned to loosen the scale and oil; after cleaning has been completed, the parts are rinsed and then overcoated as desired. The cleaning and rinsing operation is conveniently effected in an inclined rotary open end barrel, the impingement of the parts on each other and the walls of the barrel during rotation serving to loosen the scale, oil and dirt which contaminates the metal substrate. The mechanical cleaning is rendered more efficient by including small particles, or impact media, in the charge.

In a typical cleaning operation, 6 cubic feet of metal articles to be cleaned are charged to an obliquely disposed 200-gallon octagonal rotary treating barrel. To the barrel are then added 3 quarts of the cleaning solution of the example, 30 gallons of water, and 6 cubic feet of impact media (e.g., a blend of glass beads, 90% having an average diameter of 0.012 to 0.022 inch and 10% having a diameter of 0.006 to 0.007 inch). Live steam is introduced to heat the charge to near 212° F. and the barrel set in motion. After approximately 15 minutes of operation the barrel is turned to rinse position and rotated while rinse water is supplied continuously for 5 minutes at a rate of about 12 gallons per minute. The excess liquid is then decanted, and, if mechanical plating is to be carried on in the same barrel, a conventional anchoring solution (such as a coppering solution) and a mechanical plating charge are successively introduced. If, alternatively, the cleaned articles are to be painted, electroplated, or otherwise overcoated, they are screened from the impact media and transported to the next station.

In a test (described in SAE 1065-1080) for determining the hydrogen embrittling characteristics imparted by cleaning, a standard high carbon steel spring wire hose clamp having a Rockwell C hardness of at least 53 is cleaned, plated, and, after a given lapse of time, spread with a standard instrument and slipped over a bar which is slightly greater in diameter than the normal I.D. of the clamp. If the hose clamp has been hydrogen-embrittled, it will fail, i.e., break, either immediately, or within 24 hours; generally speaking, the shorter the time lapse before testing, the greater the probability of failure. A total of 150 No. 15 hose clamps were cleaned as just described, given a copper anchor coat, and immediately mechanically plated with zinc. Four hours after plating, 50 of the clamps were mounted on a test bar having a diameter of 0.953 inch, no failures occurring within 24 hours. Twenty-four hours after plating, the other 100 clamps were mounted on the test bar; again no failures occurred within 24 hours.

<sup>1</sup> Mineral spirits, or ligroin, i.e., the fourth fraction of petroleum distillation product, having a density of 0.707 to 0.722 and a boiling range of 90-120° C.

The example herein is, of course, intended to be merely illustrative, and numerous variations can be made in the practice of the invention. For instance, many acids—or blends of acids—may be employed. Mineral acids such as sulfuric and phosphoric are strong and less expensive, offering obvious economic advantages. Because such mineral acids attack even very stable surfactants in concentrated form, it is often preferred to add the acid and the remaining ingredients separately at the time of cleaning. Generally, too, the stronger inorganic acids tend to dissolve the metal at a rapid rate, and, particularly in the case of high carbon or heat-treated steel parts, a carbon smut residue often remains on the surface. This condition may be alleviated by adding a small amount of one or more soluble salts, e.g., sulfates, of tin, lead, cadmium, mercury, etc. It is also desirable under such conditions to make certain that a carbon soil dispersant, i.e., a high-HLB surfactant, is present in the surfactant mixture. Phosphoric acid, as is well known, offers particular advantages when the surface to be cleaned is thereafter to be painted. Likewise, it is convenient to use the acid salts of mineral acids (e.g., sodium bisulfate or monobasic sodium phosphate) or salts which hydrolyze to form "available" hydrogen ions (e.g., aluminum chloride or ammonium sulfate).

Many other organic acids, both monobasic and multi-basic, may be employed. For example, tartaric, citric, di-glycolic, chlorosulfonic, formic, acetic, and mono-, di- or tri-chloroacetic acid may be employed. In calculating the available hydrogen ions which an acid can supply, only those acid radicals having a dissociation constant of at least  $10^{-6}$  are considered effective. Acids which might be considered too weak are rendered more effective by the preferred elevated cleaning temperature.

Glycolic acid possesses the advantage that it is a sequestering agent and hence aids in competing with the metal for the oxygen atoms which are in the oxide coating; similarly, where the available water supply contains an ion which interferes with cleaning action, glycolic acid aids in sequestering such ions. Where it is desired to provide a sequestering agent while employing an acid which does not have this characteristic, other acid-stable sequestering agents may be added; thus, "Versenex 80" (based on a diethylene triamide penta acetic acid adduct) or "Clarotex" may be used.

The "Pluronics" are attractive surfactants to work with because their stability, chemical similarity, and physical characteristics have been determined. The surfactant mixture of the cleaning solution described herein may, however, be any acid-stable materials of suitable HLB having the following ionic nature: all anionic, a blend of anionic and non-ionic, all non-ionic, a blend of non-ionic and cationic, and all cationic. Such N,N-ethoxylated unctuous nitrogenous compounds as "Ethomeen C/25" (coco amine which is N,N-substituted with a total of 15 mols of ethylene oxide to form a cationic surfactant) or "Ethomid HT/25" (hydrogenated tallow amide which is N,N-substituted with a total of 15 mols of ethylene oxide to form a nonionic surfactant) tend to adsorb on metal surfaces, reducing the need for low HLB wetting agents and aiding in the otherwise difficult cleaning of metal articles having a thin tightly adsorbed film, e.g., of a sulfonated oil. The addition of these surfactants thus extends the usefulness of the cleaning compositions described herein.

A number of materials have been empirically found to inhibit hydrogen embrittlement. "Composition A," described in connection with the example herein, contains a combination of materials which are individually effective in this regard, both the polyoxyethylene glycol and

the o-toluidine being able to reduce or suppress hydrogen embrittlement, even at high temperatures. In "Composition A" some of these materials are reacted, resulting in an adduct of orthotoluidine and formaldehyde having the characteristics of stability and excellent inhibition. As a matter of practicality, however, a wide variety of commercially available inhibitors, such as "Polyrad 1110A," "Armohib 28," or hexynol, substituted thioureas, and most amines or proteins, can be employed with at least some degree of success. Inhibitors are at least somewhat selective, however, and a given inhibitor may be more effective with one acid than with another.

What we claim is:

1. A balanced composition for preparing a wide variety of scaly, oily, dirty, or otherwise contaminated ferrous metal surfaces for subsequent overcoating, consisting essentially of a water-soluble mixture of:

sufficient strong acid, having a dissociation constant greater than  $10^{-6}$ , to provide 1-5 parts by weight of hydrogen ion, and

an acid-stable surfactant system consisting essentially of substantially equal parts by weight of the following individually acid-stable components:

dispersant having an HLB value of at least 17, detergent having an HLB value in the range of 12-17,

sufficient emulsifier to emulsify 150 parts by weight of mineral spirits, said emulsifier having a higher molecular weight than said detergent and an HLB value in the range of 12-17, and

wetting agent for ferrous metals, the lipophilic groups being dominant in said wetting agent, having an HLB value on the order of 5 or less.

2. The composition of claim 1 wherein the wetting agent is a surfactant selected from the class consisting of coco amine N,N-substituted with ethylene oxide and hydrogenated tallow amine N,N-substituted with ethylene oxide.

3. The composition of claim 1 wherein each of the components of the surfactant system has a hydrophobic polyoxypropylene nucleus with hydrophilic polyoxyethylene chains graft-polymerized thereon.

4. A one-shot method of preparing ferrous metal articles for subsequent overcoating comprising: (1) placing in a rotary container, impact media, water, on the order of 10,000 parts by weight of small ferrous articles to be cleaned, and the composition of claim 1, (2) rotating said container to both mechanically and chemically clean, de-scale, and desmut the metal articles, and (3) removing the cleaning solution.

5. The method of claim 4 in which live steam is supplied to heat the contents of the container.

#### References Cited

##### UNITED STATES PATENTS

|           |         |                 |       |           |
|-----------|---------|-----------------|-------|-----------|
| 2,261,700 | 11/1941 | Ryznar          | ----- | 252-143 X |
| 2,326,837 | 8/1943  | Coleman         | ----- | 252-142   |
| 2,399,267 | 4/1946  | Szatyn          | ----- | 134-28    |
| 2,571,581 | 10/1951 | Kearney         | ----- | 134-33 X  |
| 2,683,343 | 7/1954  | Gellette et al. | ----- | 134-7 X   |
| 2,942,956 | 6/1960  | Kelly           | ----- | 134-3 X   |
| 3,041,285 | 6/1962  | Newman          | ----- | 134-3 X   |
| 3,162,547 | 12/1964 | Kendall         | ----- | 134-41 X  |

LEON D. ROSDOL, Primary Examiner.

ALBERT T. MEYERS, Examiner.

M. WEINBLATT, Assistant Examiner.